

Patented Sept. 1, 1925.

1,552,184

# UNITED STATES PATENT OFFICE.

NATHAN H. ADAMS, OF SCHENECTADY, NEW YORK, ASSIGNOR TO GENERAL ELECTRIC COMPANY, A CORPORATION OF NEW YORK.

## METAL COMPOSITION AND METHOD OF MANUFACTURE.

No Drawing.

Application filed December 31, 1924. Serial No. 759,213.

To all whom it may concern:

Be it known that I, NATHAN H. ADAMS, a citizen of the United States, residing at Schenectady, in the county of Schenectady, 5 State of New York, have invented certain new and useful Improvements in Metal Compositions and Methods of Manufacture, of which the following is a specification.

The present invention comprises a metal 10 composition having physical properties, such as hardness and capability of resisting deformation when subjected to pressure combined with good electrical conductivity which renders them suitable for various 15 exacting uses, such for example, as an electrode for simultaneously subjecting work to both pressure and to the heating effect of an electric current, as in spot welding, and resistance heating, or as a bearing material 20 for uses involving heavy pressures. My invention also includes an improved method of making this material.

In my prior Patent, 1,477,797 of Dec. 18, 25 1923, I have described a bearing material made by pressing a mixture of a hard material, such as tungsten, and a malleable metal, such as copper, and then fusing the latter metal.

The material made in accordance with my 30 present invention is stronger, more capable of resisting higher pressure and more uniform in composition than the material described in my prior patent. Instead of being constituted by a mixture of hard material and a softer material in which the 35 particles of refractory material are bound together by the softer metal, the improved material consists of a mass of tungsten made by causing the tungsten particles to sinter 40 and form a coherent mass preliminary to the introduction of the copper or other filler metal. In other words the tungsten particles are welded or fritted to each other and the malleable metal fills the minute spaces 45 left between the tungsten particles. While the copper strengthens the mass the tungsten particles are not imbedded in a ground mass of copper. A feature of my present invention, is the introduction of the copper, 50 or other readily fusible metal into the sintered mass of tungsten in a fused state under reducing conditions and preferably materially above the melting point of the more fusible metal.

55 My invention can be illustrated with

specific reference to the formation of a tungsten-copper composition. In its preparation comminuted tungsten such as used, for example, for the preparation of lamp filaments, is shaped by pressure into suitable 60 form and then is sintered. The pressing and sintering of the tungsten powder may proceed in general by the steps described in Coolidge Patent 1,082,933 of Dec. 30, 1913, but preferably instead of sintered by 65 two steps as described in the Coolidge patent, the tungsten is sintered after the preliminary pressing operation by heating in a hydrogen furnace to a temperature at which a sintered metal mass having a porous 70 structure results, which is capable of taking up a substantial proportion of another metal. I find a preferable range of temperature for sintering to be about 1250° to 1350° C. In accordance with the Coolidge 75 patent the shaped, powdered tungsten is sintered at about 1200° C. in a furnace and then is further sintered at a higher temperature by passage of current through the tungsten. While I may proceed by this 80 method of the Coolidge patent if the second sintering by passage of current does not occur at too high a temperature, I find the single sintering in the neighborhood of 85 about 1300° C. to be preferable.

The tungsten article produced by the sintering process has a fair amount of mechanical strength and may be readily machined if desired, but it cannot withstand high 90 pressures.

As the next step in carrying out my invention, copper or other suitable metal of only moderately high fusibility which will flow readily in the presence of hydrogen is introduced in a highly fluid state into the 95 voids or pores within the body of the tungsten. Copper is fused in contact with the sintered refractory metal and preferably heated to a temperature of about 1200 to 1300° C., under non-oxidizing conditions, 100 preferably in hydrogen gas. I find that copper in the presence of hydrogen, especially when thus heated above its melting point, to render it highly fluid will very readily permeate the entire mass of sintered 105 tungsten, apparently being drawn into the mass by capillarity. Any excess of copper left on the surface may be removed by machining. The resulting composition is hard, strong and capable of resisting high pres- 110

sures and shocks. When using copper as the impregnating metal the sintered tungsten will take up about 10% by weight of the copper.

5. My improved metal composition is substantially non-deformable when subjected to high pressure during use and has a relatively high electrical and heat conductivity. It is particularly well suited for use as an 10 electrode for resistance welding, for heating rivets, or other purposes requiring simultaneous application of high currents and high mechanical pressure to the work being heated. It is also useful as a bearing 15 material for purposes requiring it to resist high pressure during use.

I have not claimed herein an electrode for heating and exerting pressure on work, this being covered by an application filed by 20 Robert T. Gillette, Serial No. 729,169, filed July 30, 1924.

What I claim as new and desire to secure by Letters Patent of the United States, is,—

25 1. The method of making a composition of hard and soft metals which consists in forming an article comprising particles of the desired refractory metal, heating said article to a temperature high enough to cause said particles to sinter into a porous 30 coherent mass having greater mechanical strength than the unsintered article and impregnating said mass with a more fusible metal.

35 2. The method of making a composition of tungsten and copper which consists in forming a mass of sintered tungsten having a porous structure and impregnating said mass with copper, the porosity of the sintered mass being chosen to take up about 10 40 per cent copper by weight.

3. The method of making a composition of tungsten and copper which consists in shaping finely divided tungsten into desired

form, heating to a temperature of about 45 1300° C., and impregnating the resulting porous sintered product with copper.

4. The method of making a composition of tungsten and copper which consists in shaping finely divided tungsten into desired 50 form, heating to a temperature of about 1300° C. and impregnating the resulting porous, sintered product with copper in a reducing atmosphere.

5. The method of making a material suitable 55 for the construction of resistance welding electrodes and bearings which consists in pressing comminuted tungsten into desired form, firing at a temperature of about 1250 to 1350° C., and introducing into contact with the resulting sintered mass copper heated above the melting point, in a hydrogen atmosphere, thereby causing the copper to permeate the tungsten body.

6. A metal composition capable of resisting 65 mechanical deformation comprising hard metal particles fritted to each other in the form of a coherent, porous structure and a softer, more fusible metal filling the voids in said structure, said material being 70 stronger than a material consisting of the same constituents in which the hard particles have not been fritted to each other.

7. A metal composition capable of resisting 75 mechanical deformation comprising tungsten particles fritted to each other into a coherent mass having minute spaces between said particles and a filling of copper in said spaces, constituting about ten per cent by weight of the tungsten, said composition being stronger than a composition in which the tungsten particles are not fritted to each other to form a coherent mass.

In witness whereof, I have hereunto set my hand this 30th day of December, 80 1924.

NATHAN H. ADAMS.